

# United States Patent Office

2,743,204

Patented Apr. 24, 1956

1

2,743,204

## PHOSPHATE METAL COATINGS

William S. Russell, Royal Oak, Mich., assignor to Parker Rust Proof Company, Detroit, Mich., a corporation of Michigan

No Drawing. Application August 28, 1952,  
Serial No. 306,961

12 Claims. (Cl. 148—6.15)

The present invention relates to improved phosphate coating compositions and methods for forming protective phosphate coatings on metallic surfaces including iron, steel, zinc and aluminum. In particular this invention is concerned with an improved solution of the coating-phosphate type, e. g., zinc, iron or manganese phosphate, which is capable of producing unusually heavy phosphate coatings in a short period of time and to the method of forming such heavy coatings on metallic surfaces. The coatings produced by the solution and method of this invention are especially useful in improving corrosion resistance and protecting the metal surface during extreme deformation of the metal such as is encountered in successive passes through drawing dies. The coatings are additionally beneficial in increasing the wear resistance of moving parts such as piston rings, gears etc.

It is now well known that the rate of formation of phosphate coatings on metallic surfaces from solutions of the coating-phosphate type, that is solutions containing a metallic ion which becomes a part of the integral coating formed on the surface, is greatly increased by the use of oxidizing or accelerating agents. Typical oxidizing agents which have been suggested include nitrates, chlorates, bromates, sulfites, nitrites, perchlorates, periodates, permanganates, etc. Solutions of the coating-phosphate type operating under conventional commercial conditions of continuous production form coatings on ferrous surfaces usually ranging in coating weight between about 50 and 600 mg./sq. ft. For corrosion resistant applications heavier coatings averaging about 1600 to 1800 mg./sq. ft. are obtained by immersion for relatively long periods of time or by special surface preparation prior to coating or both. Heretofore it has not been possible to produce coatings sufficiently heavy to serve as corrosion-resistant coatings in periods of time as low as about 10 minutes.

The principal object of the present invention is to provide an improved phosphate coating solution which is capable of producing unusually heavy phosphate coatings on metallic surfaces in short periods of time.

Another object is to provide an improved coating solution which produces heavy phosphate coatings on metallic surfaces when applied thereto either by dipping or spraying techniques.

A further object of the present invention is to provide a method for treating the surfaces of iron, steel and zinc to form a heavy phosphate coating thereon.

Still another objective is to provide an auxiliary accelerator which in combination with conventional oxidizing agents in a coating-phosphate solution greatly increases the coating weights obtainable on metallic surfaces.

Other objects and advantageous features of the invention will become apparent upon considering the present disclosure in its entirety.

In accordance with this invention, it has been found that aqueous acidic phosphate solutions of the coating-phosphate type and having a pH in the range of 1.9 to 3.5

2

are unexpectedly accelerated by the addition thereto of small quantities of certain organic chelating agents.

Certain amino acids, and particularly alpha amino acids, such as glycine, alanine and sarcosine, form complexes with certain metal ions such as iron, copper, zinc, nickel, etc., in solution and this complexing effectively removes such ions from the solution or prevents them from carrying out their normal reactions. Polycarboxylic alpha amino acids, such as ethylenediamine tetraacetic acid, have even greater tendencies to form stable complexes or chelates with metallic ions in comparable solutions than do the simpler amino acids. Aqueous solutions of polycarboxylic alpha amino acids are alkaline in nature and are known to lose their chelating or complexing ability with decreasing pH or in other words, increasing acidity. Thus, the extra heavy coating weights, which were obtained and caused by the addition of minor quantities of such organic chelating agents to relatively acid coating-phosphate solutions were not expected, and the cause for the tremendous increase in coating weight is not completely understood. Coating weights resulting from the presence in the coating solution of small quantities of polycarboxylic amino acids have been increased by as much as ten times over that which is obtained under identical processing conditions except for the presence of the amino acid. In zinc phosphate solutions having a pH between 1.9 and 3.5, the heavy coating weights characteristic of this invention are not obtained in the absence of a conventional oxidizing agent. Manganese and iron phosphate solutions, on the other hand, do not require a conventional oxidizing agent to be present in order to obtain the extra heavy coatings in a short period of time.

Organic chelating agents which have been found to be particularly suitable for the purposes of this invention are the polycarboxylic alpha amino acids as exemplified by ethylene diamine tetra acetic acid, triglycine (the tri-acetic acid substitution product of ammonia) and the tetra acetic acid derivative of trimethylenediamine. The chelating agents may be added to the coating baths of this invention in the form of the amino acids but for solubility reasons it is preferred that the salts of the amino acids be employed, e. g. the alkali metal salts such as the sodium salts. The di, tri and tetra sodium salts may be employed.

Solutions that are useful for the purposes of this invention and fall within the general classification of coating-phosphate solutions which operate in continuous production as balanced solutions having a pH between about 1.9 and 3.5, include the phosphates of zinc, manganese and iron. Solutions having a hydrogen ion concentration greater than a pH of 1.9 have a tendency to act as a pickle and to form undesirable pits on the surface of the metal being coated. Coating-phosphate solutions have a tendency to form large quantities of insoluble phosphates commonly called sludge, and as the pH approaches 3.5 this tendency is greatly accentuated and renders the continuous operation of the solution extremely difficult. Maintenance of the pH of the solution between the limits of 1.9 and 3.5 is important and necessary to the successful formation of the desired heavy coatings of this invention.

Oxidizing agents which may be employed with such solutions and particularly with zinc phosphate solutions to increase the rate of coating formation on the surfaces of metals such as iron, steel, zinc and aluminum include the nitrites, chlorates, bromates, sulfites and nitro organic compounds such as m-nitrobenzene sulfonate, picric acid, etc. For convenience, the oxidizing agents are usually added as the salts, such as the sodium or other alkali metal salt. Concentrations of oxidizing agents which may be employed and within which results may be obtained with comparative ease are given below in Table I.

3  
TABLE I

| Oxidizing agent: | Percent |
|------------------|---------|
| Chlorate         | .03-5.0 |
| Bromate          | .03-.5  |
| Nitrite          | .01-.15 |
| Sulfite          | .02-.15 |

Other specific oxidizing agents which may be used are potassium iodate, sodium meta-nitrobenzene sulfonate, picric acid, hydroxylamine, etc. Typical concentrations which may be used are 0.02% to 0.5% potassium iodate, 0.03% to .5% sodium meta-nitrobenzene sulfonate, 0.01% to 0.3% picric acid and .01 to .3% hydroxylamine. The proportion given for each oxidizing agent is that proportion which causes a substantially equivalent amount of oxidizing or acceleration of the coating formation as is caused by any other oxidizing agent when present in the quantity shown. Nitrates may be used in manganese phosphate solutions at a concentration between 0.1% and 5% and may likewise be used in zinc phosphate solutions, although in certain cases they are not the most beneficial oxidizing agents with the latter solutions. When using nitrites it is preferable to maintain the temperature of the solution below about 140° F. inasmuch as the nitrite appears to react with the chelating agent and to decrease its effectiveness.

Increases in coating weight and improved resistance to corrosion have been observed to result from the addition of extremely small quantities of chelating agent to the coating solutions above described. Quantities as low as about .01% of ethylene diamine tetra-acetic acid or equivalent proportions of the tetra, tri or di sodium salts thereof, or of triglycine or the tetra-acetic acid derivative of trimethylenediamine are beneficial and produce increases in coating weight, and proportions up to about 3% of ethylene diamine tetra-acetic acid or its equivalent as the salt, may be used. The upper limit is not critical inasmuch as quantities in excess of 3% may be tolerated. The upper limit is usually determined on the basis of economy and ease of operation and proportions above about 1% have not been found to be necessary in the majority of applications. A few simple tests under operating conditions will easily establish the most desirable concentration. For example, in zinc phosphate solutions using chlorate as oxidizing agent, the preferred concentration of ethylene diamine tetra-acetic acid, based on the tetra sodium salt, is in the range of about .1% to about .3%. Proportions below about .01% ethylene diamine tetra-acetic acid have some beneficial effect, but the effect is not as pronounced as with concentrations exceeding 0.01%.

The following examples are given to illustrate in detail the improved compositions of this invention and the specific method which may be used in applying these compositions to metallic surfaces.

## Example 1

An aqueous solution was made up with the following composition:

|                 | Grams/liter |
|-----------------|-------------|
| Zinc            | 2.5         |
| Phosphoric acid | 10          |
| Sodium chlorate | 4           |

The solution operated at a pH of 2.3-3.35. Four inch by six inch cold rolled steel panels were cleaned of oil and other foreign material by conventional cleaning methods such as dry wiping followed by wiping in mineral spirits or a short pickle in 10% sulfuric acid. The panels were then immersed in a solution of the above composition heated to 160° F.-200° F. for periods of 1, 3, 5, 10 and 15 minutes. Coating weights received were 108 mg./sq. ft. after one minute, 110 mg./sq. ft. after three minutes and only 118 mg./sq. ft. after 15 minutes. The solution was then altered by adding .5 grams/liter of tetra sodium ethylene diamine tetra-acetate. A series of identi-

cally cleaned panels were then immersed in the new solution for 1, 3, 5, 10 and 15 minutes. Coating weights obtained increased as follows:

| Time:      | Coating weight—mg./sq. ft. |
|------------|----------------------------|
| 1 minute   | 320                        |
| 3 minutes  | 996                        |
| 5 minutes  | 1296                       |
| 10 minutes | 1364                       |
| 15 minutes | 1504                       |

The concentration of tetra sodium ethylene diamine tetra-acetate was increased to 1%, .3%, .5%, 1%, 2% and 3% and a series of panels immersed in each solution for comparable time intervals. Coating weights obtained after three minutes in each of the solutions are as follows:

| Tetra sodium ethylene diamine tetra-acetate | Coating wt., Mg./sq. ft. |
|---------------------------------------------|--------------------------|
| .1%                                         | 620                      |
| .3%                                         | 1,038                    |
| .5%                                         | 1,042                    |
| 1%                                          | 1,220                    |
| 2%                                          | 816                      |
| 3%                                          | 684                      |

Somewhat heavier coatings were obtained on steel panels preliminarily subjected to a five-minute pickle in 10% sulfuric acid solution at 180° F., but in general the preliminary treatment is unimportant so long as the surface is free of oil, grease, scale and the like.

The panels resulting from treatment in the solution containing the chelating agent were found to have superior corrosion resistance to conventional zinc phosphate coated surfaces, and to be able to withstand successive heavy draws without the need of processing between draws.

## Example 2

|                           | Grams/liter |
|---------------------------|-------------|
| Zinc dihydrogen phosphate | 18          |
| Sodium bromate            | 5.5         |

The solution operated at a pH of 2.7-2.9.

Preliminarily cleaned cold rolled steel panels were immersed in the solution heated to about 170° F. for three minutes. Coating weights averaging 55 mg./sq. ft. were obtained. To the solution was then added 2.5 grams/liter of the tetra sodium salt of ethylene diamine tetra-acetic acid, and coating weights were observed to increase to an average of 313 mg./sq. ft. after otherwise identical treatment.

A series of compositions similar to those of Example 1 and 2 were made up in which the sodium chlorate and sodium bromate was replaced with other oxidizing agents including sodium nitrate, sodium nitrite, sodium sulfite, nitrobenzene sulfonate, hydroxylamine, etc. A few of these variations are given in the following examples.

## Example 3

|                                | Grams/liter |
|--------------------------------|-------------|
| Manganese dihydrogen phosphate | 20          |
| Sodium nitrate                 | 10          |
| Triglycine                     | 5 to 30     |

## Example 4

|                                    | Grams/liter |
|------------------------------------|-------------|
| Zinc                               | 3           |
| Phosphoric acid                    | 12          |
| Sodium m-nitrobenzene sulfonate    | 3           |
| Ethylene diamine tetra-acetic acid | .4 to 27    |

## Example 5

|                                             | Grams/liter |
|---------------------------------------------|-------------|
| Manganese dihydrogen phosphate              | 15          |
| Sodium m-nitrobenzene sulfonate             | 6           |
| Tetra sodium ethylene diamine tetra-acetate | .5-30       |

## 5

## Example 6

## Grams/liter

|                                                  |       |
|--------------------------------------------------|-------|
| Zn(H <sub>2</sub> PO <sub>4</sub> ) <sub>2</sub> | 20    |
| Hydroxylamine                                    | .5    |
| Tetra sodium ethylene diamine tetra-acetate      | .5-10 |

## Example 7

## Grams/liter

|                                                  |       |
|--------------------------------------------------|-------|
| Zn(H <sub>2</sub> PO <sub>4</sub> ) <sub>2</sub> | 18    |
| Picric acid                                      | .75   |
| Tetra sodium ethylene diamine tetra-acetate      | .5-10 |

Corrosion resistance of the coatings appeared to be somewhat better when the coatings resulted from longer immersion periods, that is, between 10 and 15 minutes and the temperature approached the upper operating limit of 200° F., but the difference is slight and conventional coating phosphate operating temperatures are entirely satisfactory.

The processing procedure is not restricted to immersion inasmuch as good results have been obtained by spraying.

## Example 8

## Grams/liter

|                                                  |         |
|--------------------------------------------------|---------|
| Zn(H <sub>2</sub> PO <sub>4</sub> ) <sub>2</sub> | 18      |
| NaClO <sub>3</sub>                               | do      |
| Operating pH                                     | 2.5-3.0 |

Bumper bar stock, preliminarily cleaned, was sprayed for 60 seconds in the above solution at 138° F. Coating weights obtained varied from 48 to 135 mg./sq. ft. The solution was altered by adding 1 gram/liter of tetra sodium ethylene diamine tetra acetate. The solution then had a pH of 2.7 and coating weight after sixty-second spray varied between 336 and 416 mg./sq. ft.

## Example 9

## Grams/liter

|                                             |        |
|---------------------------------------------|--------|
| Manganese dihydrogen phosphate              | 20     |
| Tetra sodium ethylene diamine tetra-acetate | 1 to 6 |

Clean cold rolled steel panels processed in this solution at 205° F. to 210° F. for 10 minutes showed over 50% increase in coating weight as the result of adding 1 gram/liter of the chelating agent over that obtained without the chelating agent. The heaviest coating was obtained at 3 grams/liter of the chelating agent.

Portions of this solution were modified by incorporating proportions of various oxidizing agents within the above given ranges. Optimum concentrations of tetra sodium ethylene diamine tetra acetate are as follows:

| Oxidizing agent, percent:           | Chelating agent, percent |
|-------------------------------------|--------------------------|
| 1 nitrate                           | .02-.06                  |
| .1 nitrite                          | .03-.10                  |
| .6 chlorate                         | .03-.10                  |
| .6 sodium m-nitro benzene sulfonate | .01-.16                  |

A composition particularly useful for treating aluminum or aluminum alloy surfaces is given in Example 10.

## Example 10

## Pounds

|                            |      |
|----------------------------|------|
| Phosphoric acid (75%)      | 37   |
| Nitric acid, 42° Bé        | 71.5 |
| Zinc oxide                 | 42.5 |
| Boric acid                 | 18   |
| Hydrofluoric acid (60%)    | 16.5 |
| Sodium bifluoride          | 17   |
| Water to make 500 gallons. |      |

Aluminum alloy panels of alloys commercially designated 3S and 24S were treated in the above solution at 130° F. for about five minutes. The aluminum 3S panels having a nominal composition of 1.2% manganese, balance aluminum, formed a coating having a weight of 612 mgs. per square foot. The 24ST panels having a nominal composition of .8% manganese, .8% silicon and 4.5% copper, balance aluminum, in the same solutions

75

## 6

formed a coating having a weight of 367 mgs. per square ft. Various portions of the basic solution were altered by incorporating minor quantities of tetra sodium ethylene diamine tetra-acetate to produce concentrations of .03%, .06%, .1%, .3% and .6%. Increases in coating weight were observed at each concentration with a coating weight of about 1,550 mgs. per square foot occurring at .6% tetra sodium ethylene diamine tetra-acetate. Panels of 24ST stock were also treated in the alternating portions of the basic solution and comparable increases in coating weight were observed at each concentration up to a maximum of about 1,840 mgs. per square foot at .6% concentration of tetra sodium ethylene diamine tetra-acetate. The most desirable concentration of tetra sodium ethylene diamine tetra-acetate in this solution appears to be between .3% and .6%.

A solution particularly adapted for coating zinc, galvanized iron or the like is given in Example 11.

## Example 11

## Grams/liter

|                   |    |
|-------------------|----|
| Zinc              | 3  |
| PO <sub>4</sub>   | 10 |
| Nickel            | 3  |
| NaBF <sub>4</sub> | 3  |
| NO <sub>3</sub>   | 3  |

The aqueous solution having the above analysis is preferably formed by admixing proportions of salts of the various components such as nickel sulfate, nickel nitrate and zinc dihydrogen phosphate in preliminarily calculated quantities. Ordinary galvanized panels were processed in this solution at 150° F. for five minutes, and an average coating weight of 445 mgs. per square foot was obtained. Portions of the solution were modified by incorporating quantities of tetra sodium ethylene diamine tetra-acetate to produce concentrations of .03%, .06%, .1%, .3% and .6%. The coating weights were noted to increase from the lowest quantities upward to a maximum of about 2,650 mgs. per square foot at a concentration of .6% of the tetra sodium ethylene diamine tetra-acetate. The optimum operating concentration of tetra sodium ethylene diamine tetra-acetate lies between .3% and .6%.

What is claimed is:

1. A solution for producing phosphate coatings on metallic surfaces consisting essentially of a phosphate of a metal selected from the group consisting of iron, zinc and manganese, and an acetic amino acid, said solution having a pH in the range of about 1.9 and 3.5.
2. A composition for producing heavy phosphate coatings on metallic surfaces in short periods of time which consists essentially of an aqueous acidic solution of a phosphate of a metal from the group consisting of iron, zinc and manganese, an oxidizing agent and an acetic amino acid, said solution having pH in the range of 1.9 to 3.5.
3. A solution for producing heavy phosphate coatings on metallic surfaces in short periods of time consisting essentially of an aqueous acidic solution of a phosphate selected from the group consisting of zinc phosphate, iron phosphate and manganese phosphate, an oxidizing agent selected from the group consisting of nitrates, nitrites, chlorates, bromates, sulfites, nitrobenzene sulfonate, picric acid, and hydroxylamine, and an acetic amino acid, said solution having a pH between 1.9 and 3.5.
4. A solution for producing heavy phosphate coatings on metallic surfaces in short periods of time consisting essentially of an aqueous acidic solution of a phosphate selected from the group consisting of zinc phosphate, iron phosphate and manganese phosphate, an oxidizing agent selected from the group consisting of nitrates, nitrites, chlorates, bromates, sulfites, nitrobenzene sulfonate, picric acid, and hydroxylamine, and at least about .01% of ethylene diamine tetra-acetic acid, said solution having a pH between 1.9 and 3.5.
5. A solution for producing heavy phosphate coatings

on metallic surfaces in short periods of time consisting essentially of an aqueous acidic solution of a phosphate selected from the group consisting of zinc phosphate, iron phosphate and manganese phosphate, an oxidizing agent selected from the group consisting of nitrates, nitrites, chlorates, bromates, sulfites, nitrobenzene sulfonate, picric acid, and hydroxylamine, and a chelating agent selected from the group consisting of ethylene diamine tetra-acetic acid, triglycine, the tetra-acetic acid derivative of trimethylene diamine and the alkali metal salts thereof in an amount equivalent to .01% to 3% of ethylene diamine tetra-acetic acid, said solution having a pH between 1.9 and 3.5.

6. A solution for producing heavy phosphate coatings on metallic surfaces in short periods of time consisting essentially of an aqueous acidic solution of a phosphate selected from the group consisting of zinc phosphate, iron phosphate and manganese phosphate, an oxidizing agent selected from the group consisting of nitrates, nitrites, chlorates, bromates, sulfites, nitrobenzene sulfonate, picric acid, and hydroxylamine, and about .01% to about 3% of ethylene diamine tetra-acetic acid, said solution having a pH between 1.9 and 3.5.

7. A method which comprises obtaining a corrosion resistant heavy coating on iron, steel and zinc by subjecting the surface of said metal to the action of an aqueous acidic solution of a phosphate of a metal from the group consisting of iron, zinc and manganese; and an acetic amino acid, the pH of the said solution being between 1.9 and 3.5.

8. A method which comprises obtaining a heavy, corrosion resistant coating on a metal selected from the group consisting of iron, steel and zinc by subjecting the surface of said metal to the action of an aqueous acidic solution of a phosphate selected from the group consisting of zinc phosphate, iron phosphate and manganese phosphate, an oxidizing agent selected from the group consisting of nitrates, nitrites, chlorates, bromates, sulfites, nitrobenzene sulfonate, picric acid, and hydroxylamine, and an acetic amino acid, said solution having a pH between 1.9 and 3.5.

9. A method which comprises obtaining a heavy, corrosion resistant coating on a metal selected from the group consisting of iron, steel and zinc by subjecting the surface of said metal to the action of an aqueous acidic solution of a phosphate and manganese phosphate, an oxidizing agent selected from the group consisting of nitrates, nitrites, chlorates, bromates, sulfites, nitrobenzene sulfonate, picric acid, and hydroxylamine, and at least about .01% of ethylene diamine tetra-acetic acid, said solution having a pH between 1.9 and 3.5.

10. A method which comprises obtaining a heavy, corrosion resistant coating on a metal selected from the group consisting of iron, steel and zinc by subjecting

the surface of said metal to the action of an aqueous acidic solution of a phosphate selected from the group consisting of zinc phosphate, iron phosphate and manganese phosphate, an oxidizing agent selected from the group consisting of nitrates, nitrites, chlorates, bromates, sulfites, nitrobenzene sulfonate, picric acid, and hydroxylamine, and a chelating agent selected from the group consisting of ethylene diamine tetra-acetic acid, triglycine, the tetra-acetic acid derivative of trimethylene diamine and the alkali metal salts thereof in an amount equivalent to .01% to 3% of ethylene diamine tetra-acetic acid, said solution having a pH between 1.9 and 3.5.

11. A method which comprises obtaining a heavy, corrosion resistant coating on a metal selected from the group consisting of iron, steel and zinc by subjecting the surface of said metal to the action of an aqueous acidic solution of a phosphate selected from the group consisting of zinc phosphate, iron phosphate and manganese phosphate, an oxidizing agent selected from the group consisting of nitrates, nitrites, chlorates, bromates, sulfites, nitrobenzene sulfonate, picric acid, and hydroxylamine, and about .01% to about 3% of ethylene diamine tetra-acetic acid, said solution having a pH between 1.9 and 3.5.

12. A composition for producing heavy phosphate coatings on metallic surfaces in short periods of time which consists essentially of an aqueous acidic solution of a phosphate of a metal from the group consisting of iron, zinc and manganese, an oxidizing agent, a fluoride and an acetic amino acid, said solution having a pH in the range of 1.9 to 3.5.

#### References Cited in the file of this patent

#### UNITED STATES PATENTS

|           |                       |               |
|-----------|-----------------------|---------------|
| 1,911,726 | Tanner et al. -----   | May 30, 1933  |
| 2,132,883 | Romig -----           | Oct. 11, 1938 |
| 2,298,280 | Clifford et al. ----- | Oct. 13, 1942 |
| 2,316,811 | Romig -----           | Apr. 20, 1943 |
| 2,461,519 | Bersworth -----       | Feb. 15, 1949 |
| 2,479,423 | Snyder -----          | Aug. 16, 1949 |

#### FOREIGN PATENTS

|         |                     |               |
|---------|---------------------|---------------|
| 663,650 | Great Britain ----- | Dec. 19, 1949 |
|---------|---------------------|---------------|

#### OTHER REFERENCES

"The Properties and Uses of Ethylenediamine Tetra Acetic Acid and Its Salts," published 1949 by the Bersworth Chemical Co., Framingham, Mass. Page 7 is particularly pertinent.

"The Modern Chelating Agent," published 1949 by the Bersworth Chemical Co., Framingham, Mass. Pages 1, 8-11 and 13 are pertinent.